

March 30, 1937.

C. E. K. MEES

2,075,046

PHOTOGRAPHIC EMULSION CONTAINING SUPERSENSITIZED PINACYANOL

Original Filed Nov. 4, 1932



**A** = Pinacyanol

**B** A dialkylaminostyryl derivative of  
an alkyl quaternary salt of a simple  
nitrogen-containing heterocyclic base

**C** A combination of these two dyes.

Charles E. K. Mees,  
Inventor:

Daniel J. Mayne

By Newton M. Perraud

Attorneys:

## UNITED STATES PATENT OFFICE

2,075,046

PHOTOGRAPHIC EMULSION CONTAINING  
SUPERSENSITIZED PINACYANOLCharles E. K. Mees, Rochester, N. Y., assignor, by  
mesne assignments, to Eastman Kodak Com-  
pany, Jersey City, N. J., a corporation of New  
JerseyApplication November 4, 1932, Serial No. 641,177  
Renewed February 9, 1935

10 Claims. (Cl. 95—7)

This invention relates to sensitized photo-  
graphic emulsions and more particularly relates  
to photographic emulsions such as those of the  
gelatino-silver-halide type containing a combi-  
nation of sensitizers, one of which cooperates  
with the other to sensitize the emulsion to a  
much greater degree than is possible with that  
sensitizer, or either sensitizer alone, or even than  
would be evidenced by the sum total of the sen-  
sitzation produced by the two separate sensi-  
tizers individually.

In other words, I have found that the sensi-  
tivity contributed to photographic emulsions by  
certain sensitizers may be enhanced to a very  
considerable degree by adding to the basic sen-  
sitizer what I will term a "supersensitizer", the  
latter contributing to the emulsion the sensitivity  
which is peculiar to itself as well as activating or  
inducing further sensitivity in what I will term  
the "basic sensitizer." For example, a certain  
basic sensitizer may have a green speed of 50 H  
and D, but when there is added thereto a super-  
sensitizer, which may not even sensitize to the  
green at all (but to some other portion of the  
spectrum) the green speed of the basic sensi-  
tizer will be increased far beyond its original  
green speed. Or, assuming the basic sensitizer  
to sensitize the emulsion to a green speed of 50  
and the supersensitizer to separately sensitize  
the emulsion to a green speed of 5, the addition  
of the supersensitizer to the basic sensitizer will  
sensitize the emulsion to a green speed beyond  
the sum total of the two separate green speeds,  
namely to a green speed, for instance of 80.

The combination of sensitizers and supersensi-  
tizers which are the subject of the instant in-  
vention have the peculiar property that, in order  
for the supersensitizer to increase the sensitivity  
of the basic sensitizer, the region of sensitivity of  
the supersensitizer must coincide at least in part  
with the region of sensitivity of the basic sensi-  
tizer. The unusual effects obtained by the com-  
binations of sensitizers which constitute the in-  
stant invention result, therefore, from the un-  
usual influence or relation which the supersen-  
sitzers have upon or to the respective basic sen-  
sitzers.

Accordingly, it is among the objects of my in-  
vention to provide a photographic emulsion  
which contains a basic sensitizer for the emul-  
sion and which also contains a supersensitizer  
which contributes its own individual sensitiza-  
tion to the emulsion and also increases the sen-  
sitzation caused by the basic sensitizer. It is  
a further object of my invention to provide cer-

tain combinations or mixtures of sensitizers in  
a photographic emulsion which will contribute  
to the emulsion a sensitivity (ability to respond  
to light) not heretofore obtainable with either  
of the individual sensitizers in the combination. 5  
Other objects will become apparent to those  
skilled in the art upon a further perusal of this  
specification.

I have found, for instance, that the sensitivity  
which pinacyanol contributes to a gelatino-sil-  
ver-halide emulsion will be markedly increased  
if there is present in the photographic emulsion  
along with each part of the pinacyanol, from  
approximately  $\frac{1}{16}$ th part, or even less, to approx-  
imately one part, or even more, of certain styryl  
compounds as a supersensitizer. I find this sup-  
ersensitizing effect upon the sensitizing prop-  
erties of pinacyanol to be general with or repre-  
sentative of certain styryl compounds which  
themselves have the ability of separately sen-  
sitzing photographic emulsions to some degree. 20

Referring to the attached drawing, forming a  
part hereof, there is represented a hypothetical  
wedge spectrogram illustrating my invention.  
The curve A shows the approximate sensitivity  
conferred upon a gelatino-silver-halide emulsion  
by pinacyanol as a basic sensitizer. The curve  
B illustrates diagrammatically the sensitivity  
separately conferred upon the same gelatino-sil-  
ver-halide emulsion by a styryl compound, such  
as 4 methyl 2 (p. diethylamino styryl) thiazole  
ethiodide. The curve C, however, illustrates the  
sensitivity of the same photographic emulsion  
containing a small percentage of a solution in  
which is dissolved approximately equal parts of  
pinacyanol and the same styryl compound. 30  
From this it will be apparent that the combina-  
tion or mixture of these sensitizers contributes  
to the photographic emulsion a sensitivity far  
beyond that which it is possible to obtain even  
from the sum total of the sensitization resulting  
from the individual sensitizers. 35

More specifically my invention is accomplished  
by dissolving the sensitizing dyes in, for instance,  
methyl alcohol. The sensitizer and supersensi-  
tizer are added to the alcohol, for instance, in  
equal proportions, although I have found that  
less than an equal amount of the supersensitizer  
is normally sufficient to confer upon the sensi-  
tizer an increased sensitivity. For example, 50  
while I may dissolve in the methyl alcohol sol-  
vent one part of pinacyanol, I may then add to  
the alcohol from  $\frac{1}{16}$ th part, or even less, of the  
styryl compound to one part, or even more, of  
the styryl compound, depending upon the effect 55

that is desired in the photographic emulsion. The exact ratio of the supersensitizer to the sensitizer is not particularly important, inasmuch as those skilled in the art can readily 5 determine by what ratio the greatest degree of sensitization of the basic sensitizer can be obtained.

This solution of the sensitizer and supersensitizer is then diluted with water and a volume 10 containing from a few milligrams to as much as 100 milligrams, and preferably from about 10 to 30 milligrams of the sensitizers, is then added to 1000 cc. of a gelatino-silver-halide emulsion, such as is customarily employed in the 15 art. Obviously, if the pinacyanol is greatly supersensitized by the styryl compound, less of the sensitizer combination will be necessary to obtain the desired degree of sensitization in the emulsion. The emulsion may then be coated 20 upon a transparent support as is well known in the art, either glass, cellulose nitrate or acetate, or other cellulose derivative, base being satisfactory as the support.

As further illustrating my invention, I have 25 tabulated hereinafter typical examples of styryl compounds which themselves have the power of sensitizing a photographic emulsion and also have the ability of supersensitizing the sensitizing effect of the pinacyanol on the photographic 30 emulsion. Styryl compounds which are characteristic of those which I may employ as supersensitizers for pinacyanol are as follows:

4-methyl 2 (p. diethylamino) styryl thiazole ethiodide



40 4-methyl 2 (p. dimethylamino) styryl thiazole ethiodide

4-phenyl 2 (p. dimethylamino) styryl thiazole ethiodide

45 2 (p. dimethylamino) styryl thiazole ethiodide

2 (p. dimethylamino) styryl thiazoline ethiodide

pinaflavol



These illustrate a class of styryl compounds 55 which I have found will act as supersensitizers for pinacyanol and which class may be defined as dialkylamino styryls which contain a simple heterocyclic nitrogen containing nucleus or ring which latter may be substituted, if desired, so 60 long as such substitution does not destroy the power of the styryl to separately sensitize a photographic emulsion; alkyl and aryl groups are suitable substituents. I regard a fused-on benzene ring as being without the foregoing definition as for instance in the case of a quinoline or benzothiazole nucleus.

Pinacyanol is, of course, well known in the art as a sensitizer, having the formula—



75 The basic structure and source of the super-

sensitizers above named are well known to those skilled in the art, either being set forth in the published literature, or in available patents, so that the description of their methods of preparation is unnecessary.

In addition to the above combinations of sensitizers, I have also found that a large number of combinations of other sensitizers will produce analogous results. For instance, as described in my application Serial No. 641,178, of even date, 10 the sulphur or selenium containing pseudo cyanides may be supersensitized by those styryl compounds which contain a nitrogen containing heterocyclic nucleus which may or may not have a benzene ring fused thereon. As described in 15 my application Serial No. 641,179, of even date, the sulphur or selenium containing carbocyanines may be supersensitized by the 2:2' alkyl 8 alkyl 3:4:3':4' dibenzothiocarbocyanine halides. The numerous examples set forth in those applications further illustrate the principles of my invention. 20

Other examples showing the broad application 25 of my invention could be cited but the foregoing will be sufficient to teach those skilled in the art, the manner in which my invention is carried out and the broad principle of supersensitizing basic 30 sensitizers of numerous types with compounds which themselves have separate sensitizing properties and the regions of sensitivity of which coincide at least in part with the respective regions of sensitivity of the basic sensitizers.

Numerous variations to the above invention will 35 doubtless occur to those skilled in the art and will be included in the scope of my invention as defined by the claims appended hereto, it being understood that the foregoing is merely illustrative of the manner of practicing my invention and the results to be obtained thereby.

What I claim as my invention and desire to be 40 secured by Letters Patent of the United States is:

1. A gelatino-silver-halide emulsion containing 45 two sensitizers for the emulsion, one of which is pinacyanol as a basic sensitizer and the other of which is, as a supersensitizer, a dialkylamino styryl derivative of an alkyl quaternary salt of a simple nitrogen-containing heterocyclic base.

2. A gelatino-silver-halide emulsion containing 50 two sensitizers for the emulsion, one of which is pinacyanol as a basic sensitizer and the other of which is, as a supersensitizer, a dialkylamino styryl derivative of an alkyl quaternary salt of a simple nitrogen-containing heterocyclic base which may be substituted but which has no fused-on benzene nucleus.

3. A gelatino-silver-halide emulsion containing 55 two sensitizers for the emulsion, one of which is pinacyanol and the other of which is a 2 (p. diethylamino) styryl thiazole alkhalide.

4. A gelatino-silver-halide emulsion containing 60 two sensitizers for the emulsion, one of which is pinacyanol and the other of which is 2 (p. dimethylamino) styryl thiazole ethiodide.

5. A gelatino-silver-halide emulsion containing 65 two sensitizers for the emulsion, one of which is pinacyanol and the other of which is a 4 alkyl 2 (p. dialkylamino) styryl thiazole alkhalide.

6. A gelatino-silver-halide emulsion containing 70 two sensitizers for the emulsion, one of which is pinacyanol and the other of which is 4 methyl 2 (p. diethylamino) styryl thiazole ethiodide.

7. A gelatino-silver-halide emulsion containing 75 two sensitizers for the emulsion, one of which is pinacyanol and the other of which is 4 methyl 2 (p. dimethylamino) styryl thiazole ethiodide.

8. A gelatino-silver-halide emulsion containing two sensitizers for the emulsion, one of which is pinacyanol and the other of which is 4 aryl 2 (p. dialkylamino) styryl thiazole alkhalide.
- 5 9. A gelatino-silver-halide emulsion containing two sensitizers for the emulsion, one of which is pinacyanol and the other of which is 4 phenyl 2 (p. dimethylamino) styryl thiazole ethiodide.
10. A photographic element comprising a gelatino-silver-halide emulsion containing two sensitizers for the emulsion, one of which is pinacyanol as a basic sensitizer and the other of which is, as a supersensitizer, a dialkylamino styryl derivative of an alkyl quaternary salt of a simple nitrogen-containing heterocyclic base.

CHARLES E. K. MEES.